

(No Model.)

2 Sheets—Sheet 1.

H. L. BREVOORT & I. L. ROBERTS.

SEPARATING PARTITION FOR GALVANIC BATTERIES.

No. 394,638.

Patented Dec. 18, 1888.

Fig: 1.



Witnesses:

*A. Hyatt*  
*B. T. Tetterlein.*

Inventors:

*Henry L. Brevoort,*  
*Isaiah L. Roberts,*

*by their Atty*  
*Henry L. Brevoort*

(No Model.)

2 Sheets—Sheet 2.

H. L. BREVOORT & I. L. ROBERTS.  
SEPARATING PARTITION FOR GALVANIC BATTERIES.

No. 394,638.

Patented Dec. 18, 1888.

Fig. 3.



Fig. 2.



Witnesses:

H. L. Brevoort  
B. J. Vottilain

Inventors

Henry L. Brevoort  
Isaac L. Roberts  
by their Atty  
N. L. Brevoort

# UNITED STATES PATENT OFFICE.

HENRY L. BREVOORT AND ISAIAH L. ROBERTS, OF BROOKLYN, ASSIGNORS  
TO THE ROBERTS-BREVOORT ELECTRIC COMPANY, (LIMITED,) OF NEW  
YORK, N. Y.

## SEPARATING-PARTITION FOR GALVANIC BATTERIES.

SPECIFICATION forming part of Letters Patent No. 394,638, dated December 18, 1888.

Application filed May 1, 1886. Serial No. 200,847. (No specimens.)

*To all whom it may concern:*

Be it known that we, HENRY L. BREVOORT and ISAIAH L. ROBERTS, citizens of the United States, and residents of the city of Brooklyn, county of Kings, State of New York, have invented certain Improvements in Galvanic Batteries, of which the following is a specification.

Heretofore, where it has been desired to use two different liquids in the cells of a galvanic battery, porous partitions of earthenware have been employed to separate the liquids from each other. To accomplish the separation only, a non-porous partition would have been preferable; but such a partition would have been useless, because it would have cut off the electrolytic liquids or solutions from contact with each other. This contact has heretofore been secured by having the partition porous, so that the liquids penetrating the pores of the partition could form lines or chains of electrolytic molecules, through which the electrolytic action or energy could be transmitted. The solid portion of the porous partition of course offers an absolute resistance to the transfer of electric action, which is transmitted solely by the electrolysis of the liquid or liquids held in the pores. To reduce the total resistance of the partition, it was therefore desirable or necessary to have its porosity very great. Any porous body will, however, allow or even promote the transfusion of liquids through it, and therefore such transfusion always took place where porous partitions were used and was a necessary though undesirable result of their constitution and mode of action. In other words, the porous partition was itself impotent as a means of transmitting the electric force, and only acted as a frame-work to hold the molecules of the electrolytic liquid or liquids which transmitted the electric force by their successive decompositions and recombinations. The electrolytic liquids, however, by reason of their liquid character, tended to diffuse and mingle, and this tendency was restrained by the porous body only to a limited degree. To illustrate this: If a solution of sulphate of copper be placed outside an ordinary porous cup and sulphate of zinc on the inside, in a

few hours, or perhaps in a day, a large portion of the sulphate of copper will have intermixed with the sulphate of zinc, and a large portion of the sulphate of zinc will have passed through the porous cup into the sulphate-of-copper section. This intermixing of the fluids will of course ruin the battery by occasioning "local action."

We make the diaphragm or partition of the battery of a material which is practically non-porous, but with electrolytic properties, so that whether the battery be on an open circuit or closed the liquid, as such, on one side of the partition will not intermix or intermingle with the liquid on the other side of the partition, or only to a very limited extent; but when the circuit is closed and the battery is called upon to give a current of electricity chemical action can and will take place through the partition.

In carrying out our invention we construct the partition or diaphragm either partially or wholly of a gelatinous or jelly-like material which is non-porous, but which contains moisture as one of its characteristic elements. Thus the partition may be made of starch, preferably boiled in a strong brine of some salt of an alkali—such as chloride of sodium or a salt of zinc—and the gelatinous or jelly-like mass so produced may be confined between walls of cloth or other suitable material to form the diaphragm or partition of the battery-cell. Instead of the starch we may use boiled flour—say rice-flour, wheat-flour, or, in fact, the gelatinous substance obtained from any grain or plant. The materials which are the least soluble are to be preferred. The partition may also be made, but not to such great advantage, of dough of flour and water, which may be left unboiled and may be confined between the sustaining-walls. The thickness of the gelatinous or jelly-like mass forming the partition should be anywhere from a quarter of an inch upward, varying with the size of the battery used, though it may be of more or less thickness. The gelatinous material may be introduced into a thickness of cloth or felt by being caused to enter and close the pores thereof to form the non-porous partition, and in this case

the two retaining-walls of cloth would not be necessary. In all cases we prefer to use a salt in the gelatinous material, as it increases the electrolytic properties of the partition.

The action of our diaphragm or partition we believe to be explainable as follows: The diaphragm or partition is a non-porous substantially-solid homogeneous wall whose particles, while sufficiently solid and compact to maintain their own positions and so prevent for practical purposes any transmission of fluids through them, are yet themselves able to act as electrolytes and suffer such decompositions and recombinations as are essential to the electrolytic transmission of electric force. In other words, we have in our partition combined in the one substance the solid properties of the earthenware and the electrolytic properties of the liquid, or we may say that we have made the electrolytes solid and the partition electrolytic.

In an application for a patent filed by us on the 14th of May, 1886, Serial No. 202,198, we have described and claimed another means for carrying out our present invention by the use of gelatinous or jelly-like substances obtained from albuminous material; and in another application for patent filed by Isaiah L. Roberts on the 5th of May, 1887, Serial No. 237,259, he has described another means for carrying out the present invention by the use of mineral gelatinous substances, while in still another application filed by said Roberts May 28, 1887, under Serial No. 239,679, he has described how the diaphragms may be made by the use of a gelatinous or jelly-like substance obtained by rendering a saponified material insoluble.

When the jelly-like or gelatinous mass is held between walls, it is advantageous to stir up with it a filamentous binding material, such as hair, fur, asbestos, fibers, or cotton. This binding material is best added when the mass is being boiled. Enough of this should be used to bind the material together and avoid cracks and the like in drying. One pound of starch and six pounds of water, two pounds of chloride of sodium, and two ounces of cotton-fiber may be stirred and boiled together until cooked with satisfactory results. Cooking is accomplished when the starch-granules are broken. We may boil with the starch the salt which is to form the basis of the solution on the zinc side of the battery. Thus, if the sulphate of copper is added on one side and the sulphate of zinc on the other side, we may boil with the starch a solution of sulphate of zinc. If sulphate of copper is used on one side and chloride of sodium on the other, we prefer to boil with the substance to form the partition chloride of sodium; but to these we do not limit ourselves in any way, as sulphate of zinc would do in the majority of cases, though we prefer chloride of sodium. It is intended to use in this battery sulphate of copper and a plate of copper on one side

and sulphate of zinc on the other of the partition; but other materials may be used. Weak acids can also be used on either side to increase the conductivity of the solution or as an excitant.

The accompanying drawings show, as an example, one mode of carrying out our invention.

Figure 1 is a plan of a cell complete. Fig. 2 is a vertical section on the line  $xx$ , Fig. 1; and Fig. 3 is a vertical section taken at right angles to Fig. 2.

A is the cell. We have shown here a cell composed of two wooden boxes placed one within the other, with a layer of asphalt and rosin between. We do not, however, confine ourselves to this peculiar style of cell, as any other style may be used without departing from the principles of the invention.

B are two wooden frames, over which is stretched a cloth or canvas, C, as indicated. These frames B are fitted to the interior of the cell, and are secured in said cell at a short distance apart and with the canvas-covered sides facing each other, and the space between the canvas sides is completely filled, as at D, with any one of the materials herein indicated, such as a mixture of boiled starch and cotton-fiber, for instance. Care must be taken not to leave any empty spaces between the canvas, so as to positively prevent leakage or transfusion of the liquids used in the cell.

When the cell and, of course, the frame B are of considerable size, we prefer to introduce the intermediate cross-bars, b, which form a support for the canvas to prevent it from bulging outward when gelatinous or jelly-like material is being filled in or at any subsequent period.

We wish it to be understood that we do not limit ourselves, however, to the form of supports shown, as other constructions may be used, and for small cells supports may be dispensed with.

We do not herein claim, broadly, an electric battery provided with a partition practically non-porous and adapted to keep separate the battery-liquids, but which will permit electrolytic action through it, or, broadly, a partition for an electric battery which is practically non-porous and adapted to separate the battery-liquids, but through which chemical action may take place, because we have made claim to such broad subject-matter in an application just filed, Serial No. 280,955, dated July 25, 1888, which is a division of this.

We claim as our invention—

1. A separating diaphragm or partition for an electric battery, composed of a jelly-like or gelatinous material.

2. A separating partition or diaphragm for an electric battery, having its pores closed by gelatinous material.

3. A two-fluid electric battery having a separating diaphragm or partition of gelatinous or jelly-like material obtained from vegetable growths.

4. A separating diaphragm or partition for an electric battery, composed partially or wholly of gelatinous material, combined with a salt, as and for the purpose set forth. 20
5. A separating diaphragm or partition for an electric battery, having its pores closed by a gelatinous material containing salt, substantially as described. 25
6. In an electric battery, a separating diaphragm or partition of gelatinous or jelly-like material, combined with supporting devices, substantially as described.
7. In an electric battery, a separating diaphragm or partition of gelatinous material, combined with a supporting sheet or sheets of textile material. 30
8. In an electric battery, a separating diaphragm or partition of gelatinous material
- obtained from boiled vegetable growths, substantially as described.
9. A separating diaphragm or partition for an electric battery, partially or wholly of starch, substantially as described.
10. A separating diaphragm or partition for an electric battery, of starch, supported in position by a sheet or sheets of textile fibrous materials, substantially as described.
11. A separating diaphragm or partition for an electric battery, of gelatinous material combined with binding or holding material in the form of filaments. 35

HENRY L. BREVOORT.  
ISAIAH L. ROBERTS.

Witnesses:

MARCUS S. HOPKINS,  
JOSEPH L. ATKINS.